

## UNITED STATES PATENT OFFICE

ROBERT THOMAS WOOD, OF LAKWOOD, OHIO, ASSIGNOR TO AMERICAN MAGNESIUM CORPORATION, OF PITTSBURGH, PENNSYLVANIA, A CORPORATION OF NEW YORK

## MAGNESIUM BASE ALLOYS

No Drawing.

Application filed December 23, 1930. Serial No. 504,429.

This invention relates to magnesium base alloys and is directed to the preparation of alloys of this class containing tin and manganese.

5 In my copending application filed concurrently herewith, there is described and claimed a magnesium base alloy containing tin and manganese, with or without other alloying constituents, the alloy being characterized by unusual ease of working. In copending application of Harold H. Block and myself, also filed concurrently herewith, there is described and claimed a magnesium base alloy containing tin, zinc and cadmium, with 10 or without other alloying elements, such as manganese, the alloy being characterized by certain advantages therein disclosed. In the first of these alloys manganese is an essential constituent and in the second its presence is 15 optional although desirable.

The object of this invention is the provision of a commercially operable and economical method of introducing manganese into magnesium base alloys such as those disclosed 20 in the above mentioned copending applications, and other alloys containing tin.

Several methods have already been disclosed for introducing manganese into magnesium base alloys. For example, the metal 25 in the form of finely divided particles may be added directly to the molten magnesium. The latter may not safely be heated to more than 800° C. in ordinary atmosphere and even at this temperature considerable care is 30 necessary and the reaction with the atmosphere is severe. At best not more than a trifling amount of manganese can be alloyed in this way, probably not more than 0.02 per cent.

35 The molten magnesium may be heated to about 1100° C. in an inert atmosphere, for instance, argon or helium, and a substantially greater amount of manganese will alloy but this method is economically prohibitive.

40 The manganese may be alloyed with aluminum and this aluminum-manganese alloy added to molten magnesium as a rich alloy. This method has the disadvantage that all 45 subsequent alloys made by the addition of this rich alloy to magnesium will contain

aluminum and aluminum may not be desired in the particular magnesium alloy be compounded. Also the amount of manganese which can be added in this way is limited.

Where the presence of aluminum in the 50 magnesium alloy is not required or desirable, but where manganese and tin are desired, the method which I have invented and herewith disclose is of a special advantage.

55 In carrying out my method in the preferred manner I first prepare a tin manganese-rich alloy. I have found that if finely divided metallic manganese be added to molten in at about 500° C. very little alloying takes place even if the temperature is maintained for a relatively long time, but if the temperature is raised to between 500° C. and 1000° C. appreciable alloying of the manganese and tin occurs within a fairly 60 short time. By this method I have obtained 65 alloys of 80 per cent tin and 20 per cent manganese. By raising the temperature to between 1000° C. and 1600° C. I have produced alloys of 50 per cent tin and 50 per cent manganese. A simple yet desirable 70 precaution to prevent oxidation of the tin at elevated temperatures consists in sprinkling charcoal on the surface of the molten metal. This in no way interferes with the process 75 and may be skimmed off before the alloy is 80 poured into the usual "notch bar" molds.

Having prepared the proper manganese-rich alloy I add the necessary amount thereof, with or without additions of pure tin, to the molten magnesium. By this method the 85 desired amount of manganese is easily alloyed with the magnesium.

As a practical example of the application 90 of the principles herein outlined, I have heated a pot of molten tin to about 1100° C. and then added finely divided metallic manganese. The melt was covered with powder charcoal and maintained at this temperature for about 30 minutes, being stirred fairly 95 regularly. It was then allowed to cool, poured into "notch bars" and a chemical analysis made. This showed a manganese content of 21.06 per cent and a tin content of 78.94 per cent. By going to higher temper- 100

atures the content of alloyed manganese can be further increased, if desired.

I claim—

5 1. In compounding a magnesium base alloy containing tin and manganese, adding a tin-manganese alloy to molten magnesium.

10 2. The method of compounding a magnesium base alloy containing tin and manganese, which comprises heating tin to more than about 500° C., adding manganese thereto, maintaining the temperature of the melt until the manganese has substantially dissolved, and adding a suitable proportion of the resulting tin-manganese alloy to molten

15 magnesium.

In testimony whereof I hereto affix my signature.

ROBERT THOMAS WOOD.

20

25

30

35

40

45

50

55

60